

July 2, 1940.

W. C. LINTON

2,206,780

LEAK RESISTOR

Filed March 6, 1939

Fig. 1.



Fig. 2.

Inventor

William C. Linton.

## UNITED STATES PATENT OFFICE

2,206,780

## LEAK RESISTOR

William C. Linton, Washington, D. C., assignor  
to Fuse Indicator Corporation, Washington,  
D. C., a corporation of Delaware

Application March 6, 1939, Serial No. 260,154

7 Claims. (Cl. 201—76)

The present invention relates to resistor elements and the method of making the same and more particularly to the so-called leak resistors commonly used in connection with miniature indicating glow lamps for electrical fuses.

These miniature glow lamps contain a mixture of inert gases which pass electric currents between the electrodes thereof having a relatively low potential difference and when the electrodes 10 are connected in series with a leak resistance, the lamps are well suited as a practical indicator for plug fuses, cartridge fuses and indicator attachments for all types of fuses, as when the fuse element becomes blown or ruptured, the resistor 15 will provide means for resisting the flow of current through the circuit to which the fuse is applied for preventing damage in the electrical circuit at the point where the short circuit occurs and yet this resistor will permit sufficient leakage 20 of the current to cause the lamp to glow for giving or emitting a visible signal or indication as to the blown or ruptured condition of the fusible element.

It is common practice to form resistors from 25 molded materials as, for example, a material containing carbon or graphite as the conductor, a filler such as sand, clay or other finely divided insulating materials and a non-conducting binder such as shellac, phenol-condensation products, 30 thermo-plastic products of rubber and the like, all of which require heat, pressure, or heat and pressure to form these moldable materials into a homogeneous mass having the required electrical characteristics. Still further, these conventional and molded types of resistors have to 35 be treated with a highly conductive material or capped with bronze, brass or a combination of these metals at points where the conductors are to be connected or fastening elements are 40 required such as rivets, solder and the like for connecting the conductors to these molded types of resistors.

I have found that by mixing together powdered graphite, a powdered thermo-plastic condensation derivative of rubber prepared by the 45 treatment of rubber with a halide of amphoteric metal, and kaoline, that a moldable resinous powder is formed suitable for making leak resistances. A similar product is obtained if 50 chlorostannic acid, or analogous compound of an amphoteric metal, is used instead of a halide of an amphoteric metal. To render this moldable powder plastic, I add thereto a petroleum solvent which causes the rubber derivative contained 55 within this powdered mixture to become plastic

and this plastic rubber derivative will adhere to and hold the plastic graphite and kaoline together in proper spaced relation so that when the solvent completely evaporates, a resistor may be formed having the desired electrical and physical characteristics. Before the solvent is allowed to evaporate, this plastic mass can then be molded into various shapes or sizes required. In addition to the well known chemical reactions, physical and electrical characteristics of this 10 thermo-plastic rubber derivative, it has a great affinity to all kinds of metals and, therefore, if a lead wire of a glow lamp or other conductor is embedded in or attached to this plastic mass, they will adhere thereto, thereby establishing 15 a connection between these conductors and the resistor without the use of additional fastening elements. When the solvent is allowed to evaporate, a hard mass results which will not break down with age and which will bond solidly 20 to and electrically connect the graphite to the metal conductors attached thereto or embedded therein, thereby eliminating the use of heat, pressure, or heat and pressure in preparing or forming the resulting product.

It is therefore an object of the present invention to provide an electrical element having certain characteristics for adapting it for use in providing resistance in electrical systems or circuits which can be easily and readily handled; 30 molded into various shapes and sizes without heat, pressure, or heat and pressure, have a great affinity towards all kinds of metals and one which when molded or shaped into its final form bonds solidly, will not break down with 35 age, repels water and moisture, and will resist heat to a degree beyond its operating temperatures to which it is suited, that is, a leak resistance for electrical indicating fuses.

Other objects of the invention will be in part 40 obvious and in part pointed out hereinafter.

Fig. 1 is a vertical sectional view of an indicating plug fuse having my leak resistor applied thereto, and

Fig. 2 is an enlarged illustration in side elevation of one form of my leak resistor, having a portion thereof broken away and conductors connected thereto.

In carrying out my invention, I employ as a binder for the resistor a fine, sand-like powder 50 or an un-milled form of a thermo-plastic condensation derivative of rubber prepared by the treatment of rubber with a halide of an amphoteric metal or chlorostannic acid which during its preparation is formed into an emulsion 55

and thereafter steam distilled with agitation to remove the solvent contained therein whereby the same precipitates as a fine, sand-like thermo-plastic resinous powder.

5 I also employ a comminuted conductive material such as powdered graphite, and an inert material as a filler such as kaoline, which is a very pure, white clay ordinarily obtained in the form of an impalpable powder. These powdered materials are extremely fine so that no grit can be perceived by touch and are thoroughly mixed together.

10 As a specific example of this mixture for making leak resistors to be used in connection with glow lamp indicators for electrical fuses when applied to ordinary electrical or lighting circuits of 120 volts, I take one part of graphite, an equal part of the thermo-plastic resinous binder and two parts of kaoline. These powders are 15 then thoroughly mixed together and this mixture may be left in this dry, powdered state until it is desired to form the same into resistor elements.

15 In forming the resistor elements, this powdered mixture may be deposited in a recess or other cavity formed in the casing of electrical fuses or other supports to which the resistor elements are to be applied. To this dry, powdered mixture, I add a high grade petroleum solvent by 20 dropping the same thereupon until this powdered mixture becomes thoroughly saturated with the solvent, causing a resulting plastic mass. Lead wires or other conductors may then be inserted or embedded within this plastic mass or retained 25 against the same. When the solvent is allowed to completely evaporate, a resulting solid mass is formed having the lead wires or conductors permanently attached thereto.

30 These resistor elements may also be formed by placing a quantity of this powdered mixture in a bowl or other container and then mix the same with a petroleum solvent until a plastic mass is formed. Before the solvent is allowed to evaporate from this plastic mass, small parts 35 thereof may be taken from the bowl or other container and formed into the resistor element of the required size or shape or this plastic mass may be placed within a closed container to prevent the solvent from evaporating, and such container having a suitable ejecting device whereby 40 small portions of the plastic mass may be dispensed therefrom as needed. Small parts of this plastic mass may be applied to the opposing ends of lead wires or other conductors where a resistor element is required between the same and 45 when the solvent contained within this plastic mass evaporates, the lead wires or conductors will be connected together and retained in spaced relation. Also, a small part of this plastic mass 50 may be placed about the ends of a lead wire or other conductor and when the solvent evaporates, this plastic mass will adhere to the lead wire. This dry mass may then be simply placed against another lead wire or other conductor, thereby 55 establishing a leak resistance between such conductors.

60 The solvent employed is preferably benzene or toluol but other well known coal tar derivatives or petroleum solvents may be used.

65 70 Leak resistors prepared from a powdered mixture containing one part of the thermo-plastic resinous binder, one part of graphite and two parts of kaoline will have an electrical resistance rating of 50,000 ohms or more or sufficient resistance when applied to an ordinary lighting

75 circuit of 110 volts that will prevent any appreciable amount of current from passing through the circuit, but when a glow lamp indicator is connected to this circuit, the resistor will pass an infinitesimal amount or sufficient current to keep the lamp glowing. These lamps will function in electrical circuits of 110 volts having a resistance rating of anywhere between 50,000 and 650,000 ohms as electric power required to operate these lamps may be as low as .02 of a watt. Therefore, the resistors made from the above powdered mixture in the proportions as above enumerated need not all have the same constant rating, but the conductivity of the powdered mixture may be accordingly determined, over a wide range, by the proportion of the graphite employed. By thoroughly mixing this dielectric thermo-plastic resinous powder with a comminuted conductive material, particles of this mixture are caused to distribute themselves quite uniformly throughout the mass, with at least a part of them in conductive relation to each other, and, the number of particles being very great, either the law of averages so far applies as to produce substantially the same degree of conductivity in successive masses prepared in the same way and equally mixed, or the properties of the plastic and particles result in such substantially uniform distribution and arrangement of the latter, as to provide dependable uniformity of conductivity throughout a given mass or in respective masses similarly prepared.

80 The electrical resistance ratings of my resistor may be increased by reducing the amount of graphite and the amount of graphite removed can be replaced with kaoline. Obviously when applying a glow lamp indicator and resistor to high potential circuits, less graphite should be used and I have found that a mixture containing approximately 15% graphite, 25% the thermo-plastic resinous binder and 60% kaoline will produce resistors suitable for electrical circuits of 220 volts and a mixture containing 10% graphite, 25% the thermo-plastic resinous binder and 65% kaoline is required of resistors applied to electrical circuits of 660 volts. My method of preparing these leak resistors will obviously cause all succeeding resistors to greatly vary in their electrical resistance ratings but yet when using the same with indicator glow lamps for fuses, the 85 resistance and lamp will properly function over a wide range when preparing the resistors from a powdered combination in about the proportions above mentioned.

90 In the drawing, I have illustrated in Fig. 1 there of an electrical indicating plug fuse as is more particularly described in my copending application Serial No. 260,155, filed March 6, 1939, which comprises a casing 1 having a central contact 2 and a threaded contact shell 3 secured thereto. Within the explosive chamber of this casing is a fusible link 4 which is connected in series with the contact terminals 2 and 3. This casing has also formed therein a pocket in which is seated a leak resistor 5, whereby the lower end 95 of this leak resistor will contact with the inner face of the threaded metallic contact shell 3. A glow lamp 6 is also provided within the casing 1 which is utilized for designating the blown or ruptured condition of the fusible element 4. This lamp has one of its lead wires 7 connected to the central contact terminal 2 and its other lead wire 8 is embedded within the leak resistor 5. From this arrangement, it will be obvious that whereas the fusible element or link 4 is con- 100

5 nected to the contact terminals 2 and 3, the lamp 6 and resistor 5 are also connected in series with the contact terminals 2 and 3 but in parallel to the fusible element 4, whereby when the latter 10 blows, due to a short circuit within the electrical system to which the fuse is applied, the current will be directed through the lamp and leak resistor, thereby causing the lamp to glow. The lamp or leak resistor is never rendered operative 15 until after the fusible link is blown and as these leak resistors have a resistance rating of anywhere between fifty thousand and fifteen million ohms, considerable heat is generated therein after the blowing of the fusible element and 20 when current is first supplied to the lamp 6 for causing the same to strike or glow.

In applying my leak resistor to this type of indicating plug fuse, I first thoroughly mix together kaoline, graphite and the resinous binder 25 in dry, powdered form. This dry, powdered mixture can then be deposited within the opening or recess formed within the casing 1 of the fuse until the powder comes in direct contact with the inner face of the shell 3. After this powdered mixture is in direct contact with the threaded shell 3, a few drops of benzene is applied to the mixture, wherein it becomes plastic. The lead wire 8 of the lamp is then inserted 30 within this plastic mixture and when this solvent evaporates, the mixture results in a solid, flexible mass which strongly adheres to the metallic conductors 5 and 8, thereby establishing an excellent mechanical and electrical connection 35 between the two conductors, which will not break down with age or in any manner become impaired should excessive heat be later applied to the leak resistor as again would render the same plastic.

In Fig. 2 of the drawing, I have illustrated another form of preparing my leak resistor in which this dry, powdered mixture of kaoline, graphite and resinous binder is first subjected to a solvent such as benzene until it forms a plastic mass. This plastic mass may then be further formed 45 into any shape or size desired. While this resistor is in this plastic state, a lead wire 9 may have one end embedded therein or a flat contact terminal 10 may be placed thereagainst, whereby when the solvent within this plastic mass 50 evaporates, these metallic contacts 9 and 10 will strongly adhere thereto, forming an excellent mechanical and electrical connection without the aid of any mechanical or other forms of fastening or connecting elements.

55 Should this leak resistor be subjected to heat or temperatures above 200° F. it will soften and yet remain in a bonding contact with the metallic conductors. When the heat is removed and the resistor allowed to again cool, it will 60 still retain its desirable electrical and mechanical qualities. A resistor, after once being formed in the shape and size desired, may be softened by applying a solvent, such as benzene thereto, whereby conductors may be inserted therein or 65 placed in contact therewith. When the solvent is allowed to evaporate, the metallic conductors will be retained in a bonding contact therewith.

Manifestly, the construction herein shown is 70 capable of considerable modification and such modifications as come within the scope of my claims, I consider within the spirit of my invention.

I claim:

1. A leak resistance element comprising a

homogeneous mixture composed of graphite, an unmilled powdered form of a resinous reaction product comprising a thermo-plastic condensation derivative of rubber prepared by the treatment of rubber with a halide of an amphoteric metal or chlorostannic acid, and powdered kaolin, said resinous product being uniformly dispersed throughout the other materials. 5

2. A leak resistance element comprising a homogeneous mixture composed substantially of 10 one part powdered graphite, a substantially equal part of unmilled powdered form of a resinous reaction product comprising a thermo-plastic condensation derivative of rubber prepared by the treatment of rubber with a halide of an 15 amphoteric metal or chlorostannic acid, and powdered kaolin, said resinous product being uniformly dispersed throughout the other materials.

3. The subject matter of claim 2, and a metal conductor element in intimate contact with said 20 homogeneous mixture and completely adherent thereto.

4. A leak resistance element comprising a homogeneous mixture composed substantially of 25 one part powdered graphite, a substantially equal part of unmilled powdered form of a resinous reaction product comprising a thermo-plastic condensation derivative of rubber prepared by the treatment of rubber with a halide of an 30 amphoteric metal or chlorostannic acid, and substantially two parts powdered kaoline, said resinous product being uniformly dispersed throughout the other materials.

5. The method of fabricating leak resistance elements which consists in mixing together powdered graphite, kaolin, and a resinous reaction product comprising a thermo-plastic condensation derivative of rubber prepared by the treatment of rubber with a halide of an amphoteric metal or chlorostannic acid, saturating said mixture with a cold hydrocarbon of the benzene type 35 to form a plastic mass, applying the saturated plastic mass without pressure to the situs where the resistance element is required, and allowing the hydrocarbon to evaporate. 40

6. The method of fabricating leak resistor elements and attaching metallic electrical conductors thereto which consists in mixing together powdered graphite, kaoline and a thermo-plastic condensation derivative of rubber prepared by the treatment of rubber with a halide of an amphoteric metal or chlorostannic acid, saturating said powdered mixture with a cold hydrocarbon of the benzene type to form a 50 plastic mass, placing the metallic electrical conductors in intimate contact with said saturated plastic mass and allowing the hydrocarbon to evaporate whereby the metallic electrical conductors will be completely adherent thereto. 55

7. The method of fabricating leak resistance elements and attaching metallic electrical conductors thereto which consists in mixing together powdered graphite, kaoline and an unmilled thermo-plastic condensation derivative of rubber with a halide of an amphoteric metal or chlorostannic acid, applying said powdered mixture to the situs where the resistance element is required, saturating said mixture with a cold hydrocarbon of the benzene type to form a plastic mass, inserting a metallic electrical conductor within said plastic mass, and allowing the hydrocarbon to evaporate. 60 70 65

WILLIAM C. LINTON.